

[54] CONTACT MATERIAL FOR VACUUM SWITCH OF WC WITH CO-CU BINDER AND METHOD OF MAKING

[75] Inventors: **Kazuo Tazaki; Hisaji Shinohara; Akiyoshi Kikuchi; Katsuji Nagami**, all of Kawasaki, Japan

[73] Assignee: **Fuji Denki Seizo Kabushiki Kaisha**, Kamagawa-ken, Japan

[22] Filed: **Mar. 6, 1973**

[21] Appl. No.: **338,568**

[30] Foreign Application Priority Data

Mar. 7, 1972 Japan..... 47-023320

[52] U.S. Cl..... **29/182.1, 29/182.8, 75/200, 75/204**

[51] Int. Cl..... **B22f 1/00**

[58] Field of Search ..... **29/182.1, 182.8; 75/200, 75/204**

[56] References Cited

UNITED STATES PATENTS

|           |        |                     |          |
|-----------|--------|---------------------|----------|
| 3,301,673 | 1/1967 | Bridwell et al..... | 75/204   |
| 1,822,426 | 9/1931 | Welch.....          | 29/182.8 |

FOREIGN PATENTS OR APPLICATIONS

|         |        |                     |          |
|---------|--------|---------------------|----------|
| 459,854 | 1/1937 | Great Britain ..... | 29/182.8 |
| 503,995 | 4/1939 | Great Britain ..... | 29/182.8 |

Primary Examiner—Benjamin R. Padgett

Assistant Examiner—B. Hunt

Attorney, Agent, or Firm—Holman & Stern

[57] ABSTRACT

A contact material for a vacuum switch having a composition comprising from 50 to 75 percent of tungsten carbide, from 0.3 to 5 percent of cobalt, and a remainder of copper, said tungsten carbide having a finely pulverized structure of a grain size of less than 1.2 microns.

11 Claims, No Drawings

## CONTACT MATERIAL FOR VACUUM SWITCH OF WC WITH CO-CU BINDER AND METHOD OF MAKING

### BACKGROUND OF THE INVENTION

This invention generally relates to contact materials and more particularly to a type thereof which is specifically used in vacuum switches operable in a range of from 10 to 20 MVA at 3.3 KV, or from 25 to 50 MVA at 6.6 KV.

It is widely known that W-Cu alloys can be used as contacts in vacuum switches, and that contacts made of these alloys exhibit high resistance against welding of the contacts. It is also found that the contacts made of such materials can minimize the erosion of the contacts due to arcing in the vacuum switch.

Although the tungsten-copper alloys have advantageous features as described above, the material has a drawback in that its so-called "chopping level" is considerably high.

To overcome this disadvantage, W-Cu alloys containing bismuth have been proposed. However, the W-Cu-Bi alloys were found to be inferior in workability in brazing.

### SUMMARY OF THE INVENTION

Therefore, a primary object of the present invention is to provide a contact material to be used in a vacuum switch, which is operable with high reliability and has a low "chopping level."

Another object of the invention is to provide a contact material for a vacuum switch, which has a minimum range of variation in the "chopping level."

Still another object of the invention is to provide a contact material for a vacuum switch, wherein the value of current above which the contacts tend to be welded is comparable to those in the W-Cu alloys.

These and other objects of the invention can be achieved by a contact material for a vacuum switch, at a composition comprising from 50 to 75 percent of tungsten carbide, from 0.3 to 5 percent of cobalt, and a remainder of copper, said tungsten carbide having a minute pulverized structure of less than 1.2 microns.

### DETAILED DESCRIPTION OF THE INVENTION

The invention will now be described in detail with reference to the following table wherein various tungsten alloys and tungsten carbide alloys are compared with the material according to the present invention.

Table

| Composition<br>(% by weight) | Grain size<br>of WC (or W)<br>( $\mu$ ) | Interruptable<br>Current<br>(KA) | Chopping<br>level<br>(A) | Gas content<br>(ppm) |
|------------------------------|-----------------------------------------|----------------------------------|--------------------------|----------------------|
| 70W-Cu                       | 2                                       | 3.5~4.1                          | 7                        | —                    |
| 50WC-Cu                      | 0.7                                     | 1.5~3.8                          | 5                        | 200                  |
| 65WC-Cu                      | 1.2                                     | 1.4~2.1                          | 3.5                      | —                    |
| 70WC-Cu                      | 4                                       | < 1.7                            | —                        | —                    |
| 60WC-1Fe-Cu                  | 0.7                                     | 1.4~2.5                          | 3.7                      | —                    |
| 60WC-1Ni-Cu                  | 0.7                                     | 1.1~2.3                          | —                        | —                    |
| 60WC-0.3Co-Cu                | 0.7                                     | > 4.8                            | 3.6                      | 10                   |
| 70WC-5Co-Cu                  | 1.2                                     | > 4.8                            | 2.7                      | —                    |
| 75WC-5Co-Cu                  | 0.7                                     | 3.8~4.2                          | 2.3                      | —                    |
| 75WC-5Co-Cu                  | 4                                       | 1.0~3.5                          | 1.9                      | —                    |

As will be apparent from the above table, the interruptable current increases when cobalt is added, when the percentage of tungsten carbide becomes low, or

when the grain size of the tungsten carbide is made smaller. Furthermore, it will be apparent that the variable range of the interruptable current and the gas content in the alloy can be reduced by the addition of cobalt.

It is widely known that the smaller the amount of gas contained in a vacuum switch the better.

The welding current of a WC-Co-Cu alloy according to the present invention is comparably as great as that in the case of a W-Cu alloy. One reason for this is the high melting point of WC. Furthermore, the low "chopping level" of the WC-Co-Cu alloy according to the present invention can be considered to be also due to the inherent properties of the WC itself.

In view of these considerations, decreasing the content of WC excessively is not desirable, and the addition of excess cobalt is not advantageous because the cobalt reacts with tungsten carbide thereby lowering the melting point of the tungsten carbide.

Upon understanding these effects of WC and Co, various combination thereof may be considered depending on the application requirements. The present invention contemplates the provision of a contact material for a vacuum switch of greater capacities than 10 MVA at 3.3 KV, whereby the composition of the WC-Co-Cu alloy according to the present invention is adapted to be used for such an application.

Practical examples of contacts made of such materials will now be described.

### EXAMPLE 1

Pulverized tungsten carbide of approximately 1.2 microns in grain size was molded under a pressure of 0.15 ton/cm<sup>2</sup>, and then presintered in vacuum at 1,400°C. The percentage of voids in the presintered material was 55 percent by volume. The material was thereafter impregnated with 2 percent of Co-Cu alloy in vacuum at 1,300°C. The material thus obtained was machined into contacts of approximately 24 mm in diameter, and electrical performance tests were carried out thereon.

As a result, it was found that the chopping level of the contacts was 3.5A, and the interruptable current was more than 4.8 KA. The contacts were not fused together under a current of 20KA flowing therethrough.

### EXAMPLE 2

Tungsten carbide powder of 0.7-micron grain size and cobalt powder of 2-micron grain size were mixed

with a ratio of 98:2, and the resulting mixture was press-formed under a pressure of 0.2 ton/cm<sup>2</sup> and presintered in vacuum at 1,300°C. The percentage of voids

of the presintered material was 42 percent by volume. Thereafter, the presintered material was impregnated with Cu at 1,300°C in vacuum. The contact material thus obtained was formed into contacts as described in Example 1, and electrical performance tests were carried out thereon. As a result, the chopping level was found to be 2.6A, the interruptable current was 4.5 KA, and the current fusing the contacts together was found to be 30 KA.

In the practice of this invention as described above, finely pulverized tungsten carbide is used as the principal component, to which an appropriate amount of Co-Cu alloy is added, and the resulting mixture is formed into desired contacts, whereby interrupters and circuit breakers of high performance and reliability can be produced.

What we claim is:

1. A contact material for a vacuum switch consisting essentially of from about 50 to 75 percent of tungsten carbide having a finely pulverized structure of a grain size of less than 1.2 microns, from 0.3 to 5 percent of cobalt, and a remainder of copper.

2. The contact material as set forth in claim 1 wherein the tungsten carbide is about 60 percent in amount.

3. The contact material as set forth in claim 1 wherein the tungsten carbide is about 70 percent in amount.

4. The contact material as set forth in claim 1 wherein the tungsten carbide is about 75 percent in amount.

5. The contact material as set forth in claim 1 wherein the grain size of the tungsten carbide is 0.7 micron.

6. The contact material as set forth in claim 1 35

wherein the grain size of the tungsten carbide is 1.2 microns.

7. The contact material as set forth in claim 1 wherein the cobalt is about 2 percent in amount.

8. A method of producing a contact material for a vacuum switch in which a component of tungsten carbide having a finely pulverized structure of a grain size of less than 1.2 microns is press-formed and presintered into a porous structure, which is thereafter impregnated with another components of Co-Cu alloy, the ratio in amount of said components being from about 50 to 75 percent of tungsten carbide, from 0.3 to 5 percent of cobalt, and a remainder of copper.

9. The method as set forth in claim 8 wherein the tungsten carbide is press-formed and presintered in vacuum at approximately 1,400°C and is impregnated with the Co-Cu alloy in vacuum at approximately 1,300°C.

10. A method of producing a contact material for a vacuum switch in which a component of tungsten carbide having a finely pulverized structure of grain size of less than 1.2 microns is mixed with a component of cobalt to form a mixture thereof, then press-formed and presintered into a porous structure, and is thereafter impregnated with a component of copper, the ratio of said components being from about 50 to 75 percent of tungsten carbide, from 0.3 to 5 percent of cobalt, and a remainder of copper.

11. The method as set forth in claim 10, wherein the tungsten carbide is mixed with the cobalt of approximately 2-micron grain size, then press-formed and presintered in vacuum at approximately 1,300°C, and is thereafter impregnated with copper in vacuum at approximately 1,300°C.

\* \* \* \* \*